

Feb. 15, 1944.

J. F. ERVIN

2,341,704

METHOD OF DISINTEGRATING METAL INTO ABRASIVE MATERIAL

Filed Aug. 26, 1942

2 Sheets-Sheet 1

*Fig. 1.*



*Fig. 2.*



*Fig. 3.*



*Fig. 4*



Day

John F. Ervin  
Donald Howell  
Attorney

Feb. 15, 1944.

J. F. ERVIN

2,341,704

METHOD OF DISINTEGRATING METAL INTO ABRASIVE MATERIAL

Filed Aug. 26, 1942

2<sup>0</sup> Sheets-Sheet 2

*Fig. 5.*



*Fig. 6.*



*Fig. 7.*



Inventor

John F. Ervin

By

D. E. D. D.

Attorneys

## UNITED STATES PATENT OFFICE

2,341,704

METHOD OF DISINTEGRATING METAL INTO  
ABRASIVE MATERIAL

John F. Ervin, Ann Arbor, Mich.

Application August 26, 1942, Serial No. 456,231

5 Claims. (Cl. 83—91)

My invention relates to improvements in methods of shotting or disintegrating metal in the production of metal abrasive, or like, discrete material, the present invention being an improvement upon that disclosed in my U. S. Letters Patent No. 2,159,433, dated May 23, 1939; and in my copending application Serial No. 361,158, filed October 14, 1940.

The shotting of metal is an operation involving certain technical difficulties, one of same being to secure a uniform comminution of the metal so that the bulk is formed into globules or spheroids of the same desired size, while avoiding any substantial loss or wastage due to irregularly shaped fragments, and mere pulverulent or dust. Another main difficulty is to obtain a substantially perfect globular or spherical formation of the shotted particles of metal when broken up into discrete form, so as to avoid loss due to imperfect formations.

In my prior Patent No. 2,159,433, a method is disclosed utilizing a combination of separate liquid and separate vapor jets or streams into which the molten metal is discharged.

In my copending application, Serial No. 361,158, a method is disclosed consisting broadly in discharging a stream of molten metal into a closely spaced series of solid pencil-like jets of liquid, between, through and around which the molten stream passes, said liquid streams shattering and uniformly dividing the molten metal stream into drops which solidify into substantially round shape due to surface tension; also the molten stream of metal may be discharged into the angle formed between convergently meeting streams of liquid at or adjacent the line of intersection of the liquid streams, each liquid stream being maintained under regulated variable pressure.

The object of my present invention is to provide an improved and more efficient method of shotting metal, utilizing, in place of the liquid streams disclosed in my aforesaid application, a closely spaced series of jets of air, gas, vapor or steam, under pressure, into which is injected a heavier-than-air, or non-expansible liquid, under pressure, to create a combined medium having a controlled or regulated expansion, density, and velocity, thereby attaining a finer, more forceful spray permitting definite controlled uniformity in size of the comminuted metal particles, and materially reducing the consequent loss due to irregular disintegration.

Heretofore, gaseous jets, such as compressed air, vapor or steam have been used for disintegration of molten metal. The action of a jet of

such gaseous medium functions differently from a jet of non-expansible fluid. In a gaseous medium the velocity of the medium in the direction of projection as well as the expanding velocity of the gaseous medium must be taken into consideration as soon as the medium is released into the atmosphere. The large amount of kinetic energy which is active when the gaseous medium is released from the nozzle has a harsh action on the molten metal, and thus uniform disintegration which is required in a production of the shotted metal cannot be obtained. Steam or air projected under pressure sufficient for the operation has a much higher velocity than a liquid projected under the same pressure. The high velocity of a gaseous medium, in addition to the energy of expansion, does not give the desired effect in forming shotted metal and is not in any degree comparable with the results obtained by the projection of non-expanding liquid in pencil-like streams.

When shotting molten material by the projection of compressed air, gas or steam, there is a comparatively small weight of the medium projected at high velocity. This air or steam at approximately 110 pounds per square inch pressure will have a velocity when projected into the atmosphere of approximately 1000 feet per second. Due to the high velocity and to the kinetic activity of the compressed air, gas or steam an expansion takes place which creates a windage condition which blows the stream of metal and at the same time, when contacted at such high velocities, produces a tearing effect on the metal due to the absorption of the kinetic energy of the medium.

A liquid projected under the same pressure, 110 pounds per square inch, has a velocity approximating 70 feet per second. Under this condition, to deliver the same amount of energy to disintegrate the molten metal, a certain volume of liquid is required since the energy varies according to the square of the velocity. As a result, it is very difficult to properly contact the molten metal with a projected stream of either a liquid or gaseous medium when the stream is projected at sufficient energy to subdivide the molten metal into particles without having quite a percentage of the product discharged without proper disintegration.

I have found that a combination of a liquid and gaseous medium provides a range of velocities and weights which is much more efficient than obtained by using either liquid or gaseous medium projected alone, the combination medi-

um having a velocity of approximately 150 feet per second while having sufficient volume of liquid to give the stream the proper density as well as velocity to uniformly disintegrate the stream of metal which is contacted with the multiple drops.

Thus according to my invention, for the disintegration of a metal in a uniform way without creating disturbing influences which might make the molecular action impossible, a force is applied of such characteristic that the molten metal may enter therein and be acted upon thereby in semi-uniform manner. In my method the pressure of the compressed air, gas, vapor or steam introduced into the inlet of the nozzle may be varied from zero to 100 pounds per square inch, while the pressure of the heavier-than-air or non-expanding liquid supply to the inlet may be varied up to 60 pounds per square inch. By regulating these pressures using suitable valve mechanism I am able to project sprays with variable densities and velocities to effect the degree of disintegration required, the same being much more efficient than any other method known. My ejection method permits the use of a medium ranging from a rarified vapor projected in excess of 1000 feet per second for use in very fine disintegration, to and including a medium consisting of a liquid projected at velocity which may approximate only 50 feet per second for use in disintegration into larger particles; and the use of a combined gaseous and liquid medium is new in the manufacture of shotted material.

The invention will be more particularly described by the following specification with reference to the accompanying drawings, illustrating the same in exemplary working embodiments.

In said drawings—

Fig. 1 is a view diagrammatically illustrating the method utilizing my novel mixing nozzle.

Fig. 2 is an enlarged longitudinal section through the nozzle shown in Fig. 1.

Fig. 3 is an outlet end view of the nozzle showing the arrangement of the projected jets.

Fig. 4 is a vertical section on the line 4—4, Fig. 2.

Fig. 5 is a section through a modified nozzle.

Fig. 6 is an outlet end view of the nozzle shown in Fig. 5 showing one arrangement of outlet jets.

Fig. 7 is an end view of the nozzle shown in Fig. 5, but showing a different arrangement of outlet jets.

As shown in Fig. 1, the nozzle 1 receives, through pipe 2 having a valve 3 therein, a supply of compressed air, gas, vapor or steam from a suitable supply diagrammatically indicated at 4. Nozzle 1 also is connected, by a pipe 5 having a valve 6, with a supply 7 of liquid, such as water, under pressure, the liquid and gaseous mediums being combined within the nozzle, and being projected through the orificed end thereof in the form of closely adjacent streams 8. The stream of molten metal M is discharged from a trough T or the like and falls into the liquid-vapor streams 8, as indicated in Fig. 1.

Nozzle 1 may take the form shown in Fig. 2, the same consisting of a cylindrical body 1 having at one end a chamber 1a provided with an inlet 1b connected with pipe 2 which supplies the compressed air, gas or vapor or steam in quantities regulated by valve 3. Adjacent the opposite end of nozzle 1 is a chamber 1c having an inlet 1d connected with the liquid supply pipe 5, whereby the liquids under pressure are admitted in regulated quantities, by valve 6, into

the nozzle. Between the chambers 1a and 1c are arranged a series of parallel bores 1e which may be disposed in one or more horizontal rows as shown in Figs. 6 and 7, or may be arranged in the form of the letter V, as shown in Fig. 4, said bores 1e being relatively small and admitting jets of the compressed air, gas, vapor or steam from the chamber 1a into the chamber 1c. In the outer end of nozzle 1 are a series of tapering bores 1f disposed in alignment with the bores 1e, said bores 1f, each approximately fifty times the area of the bores 1e, bores 1f having their inlet ends beveled as at 1g, and bore 1f tapering towards their outer ends. In the form shown in Fig. 3 the bores 1f are arranged in V-formation and therefore the smaller portion 1e between the chambers 1a—1c would have a similar arrangement, the respective bores 1e—1f being disposed in axial alignment.

By the above arrangement, jets of compressed air, gas or steam may be emitted from the bores 1f, or liquid jets under pressure may be emitted therefrom, or a mixture of compressed air, gas, vapor, or steam in liquid may be emitted in the form of jets from bores 1f, the mixture of steam, gas or vapors and liquid being preferable since when breaking up molten metal by the projection of gas, air, steam or gas alone the medium would have comparatively small weight projected at high velocity. For example, air or steam at approximately 110 pounds per square inch pressure will have a velocity projecting into the atmosphere of approximately 1000 feet per second due to high velocity, and the kinetic activity of the compressed air, gas or steam, would create a windage condition which would blow the stream of metal, and at the same time when contacted at such high velocity, a tearing effect would be produced upon the molten metal due to the absorption of kinetic energy at the point of contact. When liquid alone is projected to deliver an equivalent amount of energy, since a liquid is many times heavier than air, steam or gas, the velocity is naturally much lower. Under an equivalent pressure of 110 pounds per square inch, the projecting velocity of a liquid would be approximately 70 feet per second, and hence to deliver the same amount of energy in order to disintegrate the bodies of molten metal, a certain volume of liquid is required since the energy varies with the square of the velocity. As a result, it is very difficult to properly contact the molten metal with a projected stream of either liquid or compressed gas when the stream is projected at sufficient energy to sub-divide the molten metal into particles without having quite a percentage of the product discharged without proper disintegration.

I have found that there is a point between the above liquid and gaseous medium velocities and weights which is more efficient, and I preferably use compressed air at approximately 100 pounds gauge pressure projected through the bores 1e and into the chamber 1c which is supplied with the liquid. Concentric with the line of projection of the gaseous streams from bores 1e are the larger bores 1f which are slightly tapering and contracted towards their outer ends and are provided with countersunk entrances 1g, which countersinking allows the air when projected through the nozzle across the chamber 1c to force entrained liquid therewith through the bores 1f at the required velocity. I have found that the most efficient velocity jet is in approximately 150 feet per second, with sufficient vol-

ume of liquid therein to give the stream proper density as well as velocity, in order to uniformly disintegrate all of the molten metal of the stream M which is contacted with the multiple streams 8, which streams may be arranged in one or more parallel rows, or may have a V-shaped formation as shown in Fig. 3.

The use of air, steam, vapor, or gas, compressed to sufficient pressure above atmospheric, and projected at a certain velocity and modified with a supply of a heavier medium which may be a liquid, a solid, or a heavier gas, creates in the combined projected stream a velocity and density which is effective and ideal for the purpose of making the proper sub-division of molten or other liquid form of metal.

According to the characteristics of air, steam or gas under pressure, a velocity is created at 100 pounds pressure approximating 2200 feet per second, while a liquid at the same pressure of 100 pounds per square inch creates a velocity of approximately 100 feet per second. By regulating these quantities and pressures, by means of the valves 3 and 6, I am able to project sprays with variable densities and velocities to effect the degree of disintegration required.

My method is an entirely new development in the disintegration of molten metals, and is much more efficient than any known method, and permits the use of high pressure air, steam or vapor which heretofore have not been used in such operation. The use of the high pressure air is not practical in any way unless it is used in the manner above described.

One of the primary advantages derived from the use of my method is due to the velocity and weight of the liquid, and to the expansion of the steam, compressed air or vapor being projected from the multiple bores 12, thereby creating two actions, one of which is forward and one of which is angular to the axis of the stream due to the expansion forces of the released gas, air or vapors. The action immediately spreads and sub-divides the molten metal M into an umbrella shape and allows it to drop quietly into the liquid. Thus the vital element of my method is its adaptability for adjustment to a balanced position with respect to velocity and density in order to create the necessary conditions which are best adapted to the particular situation.

It is necessary to have some force applied to the molten stream which is sufficient to sub-divide to disintegrate same, and at the same time the force must be as equally distributed as possible over a certain sectional area. Due to the force and the velocities of different sections of the streams it is almost impossible to obtain uniform velocities and distribution after they leave the nozzles. My method makes it possible to have a large sectional area on which the force is more nearly uniformly exerted. There is a further limitation in the use of liquid alone due to the ratio between the density and velocity, thus making it impossible to obtain the most efficient degree of sub-dividing. Thus if you increase the pressure, the impact created by the density of the medium with the velocities at these pressures, distorts the particles and interferes with their forming into spherical shot. When a gas or vapor is discharged the velocities follow the same formula, but the density of the mediums have to be considered. As a result, with an equivalent pressure the velocities vary as the square root of the relative densities. You then obtain a condition where you find a similar

situation such as above mentioned in the use of liquids. The velocity as created by the discharge at sufficient pressure to exert disintegrating force is so high that a considerable proportion of the material is broken down beyond commercial use for blasting operations.

Instead of using the form of nozzle shown in Figs. 2 and 4, a modified nozzle may be utilized shown in Figs. 5, 6 and 7. In this modification, 10 the nozzle 10 is provided with a single inner chamber 11 connected with the valved liquid supply pipe 5. At one end of the nozzle are a plurality of bores 12 connected with the valved gas pipe 2 through which jets of compressed air, gases or vapors are emitted in regulated amounts by manipulation of valve 3. In the opposite end of nozzle 10, opposite each of the bores 12, are outlet bores 13 which are each preferably fifty times the area of the bores 12. Figs. 5 and 6 indicate various other arrangements of the bores 12 and 13 which may be utilized in the nozzles 1 or 10. The gas or vapor passing through the orifices 12 are mixed in chamber 11 with the liquid supplied through the pipe 5, and the mixture then discharged through the outlet orifices 13. The facilities for regulating the pressure and supply of the liquid and of the compressed air, gases or vapor, make it possible to discharge through orifices 13 a medium with density and 20 velocity varying from vapor density and velocities, to that of liquid density and velocities. By projecting a number of these streams from the multiple orifices 13 it is possible to create a large cross-sectional area of almost uniformly applied 30 force into which may be poured the stream M of molten metal, and thereby obtain a wide degree of sub-division and at the same time have a force applied which is such that it does not distort the metal particles but allows same to freeze 40 into spherical bodies when dropped into a quenching or cooling medium.

I have found that there is practically no limit to the size of the molten stream M which can be disintegrated utilizing my method, this being 45 possible because my method may be adjusted to deliver a force through multiple orifices, and second, that this force can be delivered at varying velocities and densities. A vital feature of my method is due to the velocity of the liquid, 50 and to the expansion of the gaseous medium such as steam, air, gas or vapor after projection from the multiple ports 12 or 13 of the nozzles, same creating two actions, one of which is forward, and one of which is angular to the streams due 55 to the expansion of the gas, air or vapor when released. This expansion action immediately spreads and sub-divides the molten metal into umbrella shape, and allows same to drop quietly into the liquid; and the use of my method permits adjustment of the velocity and density of 60 the medium so that same will create the conditions which are best adapted for the particular purpose for the desired size of the shotted material.

65 I do not limit my invention to the exact forms shown in the drawings, for obviously changes may be made therein within the scope of the claims.

I claim:

1. The method of disintegrating molten metal 70 into globular abrasive material, which comprises the steps of entraining a flowing liquid in a flowing gas so as to increase the velocity of the liquid over that of pure liquid jets flowing under the same differential of pressure, discharging the resulting mixture at said velocity in the form

of a closely spaced series of pencil-like jets of controlled expansion, density and velocity, and discharging a stream of molten metal into said series of jets, the forward action of the liquid element of the jets between, through and around which the molten stream passes, thereby shattering and uniformly dividing said molten stream into drops which solidify into substantially round shape due to surface tension; and the expanding action of the gaseous element when released from the jets causing said element to spread the divided molten metal into umbrella

shape allowing same to drop quietly into a quenching medium.

2. In a method as set forth in claim 1, said liquid medium comprising water under pressure.

5 3. In a method as set forth in claim 1, said gaseous medium comprising compressed air.

4. In a method as set forth in claim 1, said gaseous medium comprising compressed vapors.

10 5. In a method as set forth in claim 1, said gaseous medium comprising steam above atmospheric pressure.

JOHN F. ERVIN.